



US005378587A

**United States Patent** [19]

Krishnamurthy et al.

[11] Patent Number: **5,378,587**[45] Date of Patent: **Jan. 3, 1995**

[54] **PHOTOGRAPHIC MATERIAL AND PROCESS COMPRISING A BICYCLIC PYRAZOLO COUPLER**

[75] Inventors: **Sundaram Krishnamurthy**, Penfield; **Stanley W. Cowan**, Rochester, both of N.Y.

[73] Assignee: **Eastman Kodak Company**, Rochester, N.Y.

[21] Appl. No.: **993,928**

[22] Filed: **Dec. 18, 1992**

[51] Int. Cl.<sup>6</sup> ..... **G03C 7/38**

[52] U.S. Cl. ..... **430/386; 430/387; 430/558**

[58] Field of Search ..... 430/558, 386, 387

[56] **References Cited**

**U.S. PATENT DOCUMENTS**

4,882,266 11/1989 Kawagishi et al. ..... 430/546  
5,066,575 11/1991 Sato et al. ..... 430/558  
5,236,819 8/1993 Kadokura et al. ..... 430/558

**FOREIGN PATENT DOCUMENTS**

0236131 4/1988 European Pat. Off. ..... 430/558  
3095450 9/1987 Japan ..... 430/558

*Primary Examiner*—Lee C. Wright

*Attorney, Agent, or Firm*—Arthur E. Kluegel

[57] **ABSTRACT**

A photographic element contains a photographic silver halide layer having associated therewith a bicyclic pyrazolo coupler having a ballast group represented by Formula (I):



wherein:

L is a divalent linking group connecting the methylene group to the remainder of the ballast group and containing at least one group selected from the group consisting of  $-\text{NR}^1\text{CO}-$ ,  $-\text{CONR}^1-$ ,  $-\text{NR}^1\text{SO}_2-$  and  $-\text{SO}_2\text{NR}^1-$ , wherein  $\text{R}^1$  is hydrogen or a substituent;

Y is a divalent linking group connecting L to Ar and containing a member selected from the group consisting of  $-\text{O}-$ ,  $-\text{S}-$ , and  $-\text{NR}^1-$  wherein  $\text{R}^1$  is hydrogen or a substituent;

Ar is an aryl group;

each  $\text{R}'$  and  $\text{R}''$  is independently a substituent, provided that at least one  $\text{R}''$  is a substituted or unsubstituted alkyl or alkoxy group having at least 10 carbon atoms; and

m and n are at least 1.

**8 Claims, No Drawings**

PHOTOGRAPHIC MATERIAL AND PROCESS  
COMPRISING A BICYCLIC PYRAZOLO  
COUPLER

FIELD OF THE INVENTION

This invention relates to novel bicyclic pyrazolo dye-forming couplers, to photographic silver halide materials and processes using such couplers and to the dyes formed therefrom. The couplers contain a fully substituted carbon at the 6-position and a ballast containing an aryl group substituted with an alkyl or alkoxy group of at least 10 carbon atoms bonded through specified groups to the pyrazolo nucleus.

BACKGROUND OF THE INVENTION

Color images are customarily obtained in the photographic art by reaction between an oxidation product of a silver halide developing agent and a dye-forming coupler. Pyrazolone couplers are useful for forming magenta dye images; however, such couplers have shortcomings with respect to color reproduction in that the unwanted absorption around 430 nm causes color turbidity. Bicyclic pyrazolo couplers, particularly pyrazolotriazole couplers, represent another class of couplers for this purpose. Examples of pyrazolotriazole couplers are described in, for example, U.S. Pat. No. 4,443,536; U.S. Pat. Nos. 1,247,493; 1,252,418; and 1,398,979; and U.S. Pat. Nos. 4,665,015; 4,514,490; 4,621,046; 4,540,654; 4,590,153; 4,822,730 and European Patents 177,765 and 119,860. One class of pyrazolotriazole couplers includes 1H-pyrazolo[3,2-c][1,2,4]triazole couplers and another includes 1H-pyrazolo[1,5-b][1,2,4]triazole couplers, such as described in European Patent 177765. While these couplers have a reduced level of unwanted absorption, the conversion of the coupler into an azomethine dye is slow and the maximum attainable density is reduced due to lower coupling efficiency.

Pyrazolotriazole couplers containing a t-butyl group at the 6-position are described in U.S. Pat. No. 4,882,266. An example of such a coupler is:



Such couplers suffer from the disadvantage of lower coupling reactivity manifested by lower contrast and Dmax as well as low speeds compared to the corresponding 6-methyl substituted analogs.

The existing products present a problem because they do not provide both acceptable reactivity, density and speed together with satisfactory photographic properties such as dye light stability color reproduction.

SUMMARY OF THE INVENTION

The present invention provides novel bicyclic pyrazolo couplers, dyes, photographic elements and processes. The photographic element comprises a support bearing at least one photographic silver halide

emulsion layer having associated therewith a dye-forming bicyclic pyrazolo-based coupler having a fully substituted carbon at the 6-position, wherein the dye-forming coupler includes a ballast fragment containing a 5 group comprising a substituted aryl group connected through a hetero group selected from the group consisting of oxy, thio, and amine, to a group containing a subgroup selected from the group consisting of carbonamide, carbamoyl, sulfonamide, and sulfamoyl, and 10 wherein the ballast link alpha to the bicyclic ring is a substituted methylene group, and further wherein said aryl group contains at least one substituted or unsubstituted alkyl or alkoxy substituent having at least 10 carbon atoms.

Photographic elements containing these couplers exhibit improved photographic properties such as dye light stability and color reproduction while maintaining satisfactory reactivity, density and speed.

DETAILED DESCRIPTION OF THE INVENTION

Suitably, the couplers of the invention contain a ballast represented by Formula I:



wherein:

L is a divalent linking group connecting the methylene group to the remainder of the ballast group and containing at least one group selected from the group consisting of  $-\text{NR}^1\text{CO}-$ ,  $-\text{CONR}^1-$ ,  $-\text{NR}^1\text{SO}_2-$  and  $-\text{SO}_2\text{NR}^1-$ , wherein  $\text{R}^1$  is hydrogen or a substituent;

Y is a divalent hetero linking group connecting L to Ar and containing a member selected from the group consisting of  $-\text{O}-$ ,  $-\text{S}-$ , and  $-\text{NR}^1-$  wherein  $\text{R}^1$  is hydrogen or a substituent;

Ar is an aryl group;

each  $\text{R}'$  and  $\text{R}''$  is independently a substituent, provided that at least one  $\text{R}''$  is a substituted or unsubstituted alkyl or alkoxy group having at least 10 carbon atoms; and

m is at least 1 and n is at least 1.

Suitably  $\text{R}'$ ,  $\text{R}''$ , and  $\text{R}^1$  may be and L may include a substituent group known in the art which typically promotes solubility, diffusion resistance, dye hue, or dye stability of the dye formed upon reaction of the coupler with the oxidized color developing agent. Preferably they can be halogen or an aliphatic residue including a straight or branched alkyl or alkenyl or alkynyl group, a heterocycle, an aralkyl group, a cycloalkyl group or a cycloalkenyl group. The aliphatic residue may be substituted with a substituent bonded through an oxygen atom, a nitrogen atom, a sulfur atom or a carbonyl group, a hydroxy group, an amino group, a nitro group, a carboxy group, an amido group, cyano or halogen. Most preferably they are hydrogen, an alkyl group, an aryl group, a carbonamido group, a sulfonamido group, a sulfone group, a thio group, a sulfoxide group, a ureido group or a multicyclic group.

At least one  $\text{R}''$  is an alkyl or alkoxy group having at least 10 carbon atoms and preferably at least 12 and most preferably at least 14 carbon atoms. "m" is 1 or 2 and "n" is 1 to 5 and typically 1 to 3.

The linking group L is a divalent group. Suitably, L, in addition to containing one of the groups specified above, may also contain a substituted or unsubstituted

alkylene, arylene, or alkylphenylene group of typically from 1 to 20 carbon atoms.

The group Y is either  $-\text{O}-$ ,  $-\text{S}-$ , or  $-\text{NR}^1-$  as specified above. Preferably, the Y group is  $-\text{O}-$ .

The group Ar is preferably a phenyl ring although hetero-ring and multi-ring groups are usable.

An embodiment of the invention is a photographic element comprising a support bearing at least one photographic silver halide emulsion layer and a dye-forming bicyclic pyrazolo coupler wherein the dye-forming coupler contains a ballast of formula I.

A typical coupler as described is represented by the formula II:



wherein:

R is a fully substituted carbon;

X is hydrogen or a coupling-off group;

Z<sup>a</sup>, Z<sup>b</sup> and Z<sup>c</sup> are independently selected from the group consisting of a substituted or unsubstituted methine group,  $=\text{N}-$ ,  $=\text{C}-$  or  $-\text{NH}-$ , provided that one of either the Z<sup>a</sup>-Z<sup>b</sup> bond or the Z<sup>b</sup>-Z<sup>c</sup> bond is a double

bond and the other is a single bond, and when the Z<sup>b</sup>-Z<sup>c</sup> bond is a carbon-carbon double bond, it may form part of an aromatic ring, and wherein at least one of Z<sup>a</sup>, Z<sup>b</sup> and Z<sup>c</sup> represents a methine group connected with the methylene group.

R may be any substituent containing a fully substituted carbon atom attached to the ring such as t-butyl, t-octyl (1,1,3,3-methylbutyl), t-pentyl, or adamantyl.

A preferred coupler according to the invention is represented by formula IIIA or IIIB:



where the variables are as described above.

Specific examples of couplers useful in the elements of the invention are:



5

5,378,587

6

-continued





Examples of substituent groups R', R'', R<sup>1</sup> and for inclusion in L include: an alkyl group which may be straight or branched, and which may be substituted, such as methyl, ethyl, n-propyl, n-butyl, t-butyl, trifluoromethyl, tridecyl or 3-(2,4-di-t-amylphenoxy) propyl; an alkoxy group which may be substituted, such as methoxy or ethoxy; an alkylthio group which may be substituted, such as methylthio or octylthio; an aryl group, an aryloxy group or an arylthio group, each of which may be substituted, such as phenyl, 4-t-butylphenyl, 2,4,6-trimethylphenyl, phenoxy, 2-methylphenoxy, phenylthio or 2-butoxy-5-t-octylphenylthio; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolylxy or 2-benzothiazolyl; cyano; an acyloxy group which may be substituted, such as acetoxy or hexadecanoxy; a carbamoyloxy group which may be substituted, such as N-phenylcarbamoyloxy or N-ethylcarbamoyloxy; a silyloxy group which may be substituted, such as trimethylsilyloxy; a sulfonyloxy group which may be substituted, such as dodecylsulfonyloxy; an acylamino group which may be substituted, such as acetamido or benzamido; an anilino group which may be substituted, such as phenylanilino or 2-chloroanilino; an ureido group which may be substituted, such as phenylureido or methylureido; an imido group which may be substituted, such as N-succinimido or 3-benzylhydantoinyl; a sulfamoylamino group which may be substituted, such as N,N-dipropylsulfamoylamino or N-methyl-N-decylsulfamoylamino.

Additional examples of substituent groups include: a carbamoylamino group which may be substituted, such as N-butylcarbamoylamino or N,N-dimethyl-carbamoylamino; an alkoxy carbonylamino group which may be substituted, such as methoxycarbonylamino or tetradecyloxycarbonylamino; an aryloxycarbonylamino group which may be substituted, such as phenoxy carbonylamino or 2,4-di-t-butylphenoxy carbonylamino; a sulfonamido group which may be substituted, such as methanesulfonamido or hexadecanesulfonamido; a carbamoyl group which may be substituted, such as N-ethylcarbamoyl or N,N-dibutylcarbamoyl; an acyl group which may be substituted, such as acetyl or (2,4-di-t-amylphenoxy)acetyl; a sulfamoyl group which may be substituted such as N-ethylsulfamoyl or N,N-dipropylsulfamoyl; a sulfonyl group which may be sub-

20 substituted, such as methanesulfonyl or octanesulfonyl; a sulfinyl group which may be substituted, such as octanesulfinyl or dodecylsulfinyl; an alkoxy carbonyl group which may be substituted, such as methoxycarbonyl or butyloxycarbonyl; an aryloxycarbonyl group  
25 which may be substituted, such as phenoxy carbonyl or 3-pentadecyloxycarbonyl; an alkenyl group carbon atoms which may be substituted; a carboxyl group which may be substituted; a sulfo group which may be substituted; hydroxyl; an amino group which may be  
30 substituted; or a carbonamido group which may be substituted.

Substituents for the above substituted groups include halogen, an alkyl group, an aryl group, an aryloxy group, a heterocyclic or a heterocyclic oxy group, cyano, an alkoxy group, an acyloxy group, a carbamoyloxy group, a silyloxy group, a sulfonyloxy group, an acylamino group, an anilino group, a ureido group, an imido group, a sulfonylamino group, a carbamoylamino group, an alkylthio group, an arylthio group, a heterocyclic thio group, an alkoxy carbonylamino group, an aryloxy carbonylamino group, a sulfonamido group, a carbamoyl group, an acyl group, a sulfamoyl group, a sulfonyl group, a sulfinyl group, an alkoxy carbonyl group, an aryloxy carbonyl group, an alkenyl group, a carboxyl group, a sulfo group, hydroxyl, an amino group or a carbonamido group.

Generally, the above groups and substituents thereof which contain an alkyl group may include an alkyl group typically having 1 to 16 carbon atoms. The above groups and substituents thereof which contain an aryl group may include an aryl group typically having 6 to 10 carbon atoms, and the above groups and substituents which contain an alkenyl group may include an alkenyl group typically having 2 to 20 carbon atoms.

55 The bicyclic pyrazolo contains in the coupling position, represented by X in formulas II, IIIA and IIIB, hydrogen or a coupling-off group also known as a leaving group.

60 Coupling-off groups are known to those skilled in the art. Such groups can determine the equivalency of the coupler, can modify the reactivity of the coupler, or can advantageously affect the layer in which the coupler is coated or other layers in the element by performing, after release from the coupler, such functions as development inhibition, development acceleration, bleach inhibition, bleach acceleration, color correction, and the like. Representative classes of coupling-off groups include halogen, particularly chlorine, bromine, or fluo-

rine, alkoxy, aryloxy, heterocyclyoxy, heterocyclic, such as hydantoin and pyrazolo groups, sulfonyloxy, acyloxy, carbonamido, imido, acyl, heterocyclylimido, thiocyanato, alkylthio, arylthio, heterocyclylthio, sulfonamido, phosphonyloxy and arylazo. They are described in, for example, U.S. Pat. Nos. 2,355,169; 3,227,551; 3,432,521; 3,476,563; 3,617,291; 3,880,661; 4,052,212 and 4,134,766; and in U.K. patents and published application numbers 1,466,728; 1,531,927; 1,533,039; 2,006,755A and 2,017,704A; the disclosures of which are incorporated herein by reference.

Examples of specific coupling-off groups are Cl, F, Br, —SCN, —OCH<sub>3</sub>, —OC<sub>6</sub>H<sub>5</sub>, —OCH<sub>2</sub>C(=O)NHCH<sub>2</sub>OH, —OCH<sub>2</sub>C(=O)NHCH<sub>2</sub>CH<sub>2</sub>OC(=O)OCH<sub>3</sub>, CH<sub>2</sub>OCH<sub>3</sub>, —OCH<sub>2</sub>C(=O)NHCH<sub>2</sub>CH<sub>2</sub>OC(=O)OCH<sub>3</sub>, —NHSO<sub>2</sub>CH<sub>3</sub>, —OC(=O)C<sub>6</sub>H<sub>5</sub>, —NHC(=O)C<sub>6</sub>H<sub>5</sub>, OSO<sub>2</sub>CH<sub>3</sub>, —P(=O)(OC<sub>2</sub>H<sub>5</sub>)<sub>2</sub>, —S(CH<sub>2</sub>)<sub>2</sub>CO<sub>2</sub>H,



20  
25



and



35 Preferably, the coupling-off group is H or halogen, and more preferably, H or Cl.

Suitable L groups include, for example, the following:



45 wherein: p is an integer of 1-6; m is 0, 1 or 2; each R<sup>a</sup> may be the same or different, and represents a hydrogen atom or a substituent; and Ar represents a substituted or unsubstituted arylene group (for example, a 1,4-phenylene group, a 1,3-phenylene group, a 2,7-naphthylene group, etc. Representative Ar groups (for L) include the following:



65



Bicyclic pyrazolo couplers as described can be used in ways and for purposes that such couplers have been used in the photographic art.

Typically, the coupler is incorporated in a silver halide emulsion and the emulsion coated on a support to form part of a photographic element. Alternatively, the coupler can be incorporated at a location adjacent to the silver halide emulsion where, during development, the coupler will be in reactive association with development products such as oxidized color developing agent. Thus, as used herein, the term "associated" signifies that the coupler is in the silver halide emulsion layer or in an adjacent location where, during processing, the coupler is capable of reacting with silver halide development products.

The photographic elements can be single color elements or multicolor elements. Multicolor elements contain dye image-forming units sensitive to each of the three primary regions of the spectrum. Each unit comprises a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprising at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler, at least one of the couplers in the element being a coupler of this invention. The element can contain additional layers, such as filter layers, interlayers, overcoat layers, subbing layers, and the like.

The magenta coupler of the invention may be used to replace all or part of the magenta layer image coupler or may be added to one or more of the other layers in a color negative photographic element comprising a support bearing the following layers from top to bottom:

- (1) one or more overcoat layers containing ultraviolet absorber(s);
- (2) a two-coat yellow pack with a fast yellow layer containing "Coupler 1": Benzoic acid, 4-chloro-3-((2-(4-ethoxy-2,5-dioxo-3-(phenylmethyl)-1-imidazolidinyl)-3-(4-methoxyphenyl)-1,3-dioxo-propyl)amino)—, dodecyl ester and a slow yellow layer containing the same compound together with "Coupler 2": Propanoic acid, 2-[[5-[[4-[2-[[2,4-bis(1,1-dimethylpropyl)phenoxy]acetyl]amino]-5-[(2,2,3,3,4,4,4-heptafluoro-1-oxobutyl)amino]-4-hydroxyphenoxy]-2,3-dihydroxy-6-[(propylamino)carbonyl]phenyl]thio]-1,3,4-thiadiazol-2-yl], methyl est and "Coupler 3": 60 1-((dodecyloxy)carbonyl)ethyl(3-chloro-4-((3-(2-chloro-4-((1-tridecanoylethoxy) carbonyl)anilino)-3-oxo-2-((4)(5)(6)-(phenoxy)carbonyl)-1H-benzotriazol-1-yl)propanoyl)amino))benzoate;
- (3) an interlayer containing fine metallic silver;
- (4) a triple-coat magenta pack with a fast magenta layer containing "Coupler 4": Benzamide, 3-(2-(2,4-bis(1,1-dimethylpropyl)phenoxy)-1-oxobutyl)amino)-

)amino)-N-(4,5-dihydro-5-oxo-1-(2,4,6-trichlorophenyl)-1H-pyrazol-3-yl)—, "Coupler 5": Benzamide, 3-((2-(2,4-bis(1,1-dimethylpropyl)phenoxy)-1-oxobutyl)amino)-N-(4',5'-dihydro-5'-oxo-1'-(2,4,6-trichlorophenyl)(1,4'-bi-1H-pyrazol)-3'-yl)—, "Coupler 6": Carboxylic acid, (6-((3-(dodecyloxy)propyl)amino)carbonyl)-5-hydroxy-1-naphthalenyl)—, 2-methylpropyl ester, "Coupler 7": Acetic acid, ((2-((3-((3-(dodecyloxy)propyl)amino)carbonyl)-4-hydroxy-8-((2-methylpropoxy)carbonyl) amino)-1-naphthalenyl)oxy)ethyl)thio)—, and "Coupler 8" Benzamide, 3-((2-(2,4-bis(1,1-dimethylpropyl)phenoxy)-1-oxobutyl)amino)-N-(4,5-dihydro-4-((4-methoxyphenyl)azo)-5-oxo-1-(2,4,6-trichlorophenyl)-1H-pyrazol-3-yl)—; a mid-magenta layer and a slow magenta layer each containing "Coupler 9": 2-Propenoic acid, butyl ester, styrene, 2:1:1 polymer with (N[1-(2,4,6-trichlorophenyl)-4,5-dihydro-5-oxo-1H-pyrazol-3-yl]-2-methyl-2-propenamide); and "Coupler 10": Tetradecanamide, N-(4-chloro-3-((4-((2,2-dimethyl-1-oxopropyl)amino)phenyl)azo)-4,5-dihydro-5-oxo-1-(2,4,6-trichlorophenyl)-1H-pyrazol-3-yl)amino)phenyl)—, in addition to Couplers 3 and 8;

- (5) an interlayer;
- (6) a triple-coat cyan pack with a fast cyan layer containing Couplers 6 and 7; a mid-cyan containing Coupler 6 and "Coupler 11": 2,7-Naphthalenedisulfonic acid, 5-(acetylamino)-3-((4-(2-((3-(2,4-bis(1,1-dimethylpropyl)phenoxy)propyl)amino)carbonyl)-4-hydroxy-1-naphthalenyl)oxy)ethoxy)-phenyl)azo)-4-hydroxy—, disodium salt; and a slow cyan layer containing Couplers 2 and 6;
- (7) an undercoat layer containing Coupler 8; and
- (8) an antihalation layer.

In a color paper format, the magenta coupler of the invention may suitably be used to replace all or a part of the magenta coupler in a photographic element such as one comprising a support bearing the following from top to bottom:

- (1) one or more overcoats;
- (2) a cyan layer containing "Coupler 1": Butanamide, 2- (2,4-bis (1,1-dimethylpropyl) phenoxy) -N-(3,5-dichloro-2-hydroxy-4-methylphenyl)—, "Coupler 2": Acetamide, 2-(2,4-bis (1,1-dimethylpropyl)-phenoxy)-N-(3,5-dichloro-2-hydroxy-4—, and UV Stabilizers: Phenol, 2-(5-chloro-2H-benzotriazol-2-yl)-4,6-bis(1,1-dimethylpropyl)—; Phenol, 2-(2H-benzotriazol-2-yl)-4-(1,1-dimethylpropyl)—; Phenol, 2-(2H-benzotriazol-2-yl)-4-(1,1-dimethylpropyl)-6-(1-methylpropyl)—; and Phenol, 2-(2H-benzotriazol-2-yl)-4,6-bis(1,1-dimethylpropyl)— and a poly(t-butylacrylamide) dye stabilizer;
- (3) an interlayer;
- (4) a magenta layer containing "Coupler 3": Octanamide, 2-[2,4-bis(1,1-dimethylpropyl)phenoxy]-N-[2-(7-chloro-6-methyl-1H-pyrazolo[1,5-b][1,2,4]triazol-2-yl)propyl]— together with 1,1'-Spirobi (1H-indene), 2,2', 3,3'-tetrahydro-3,3',3'-tetramethyl-5,5',6,6'-tetrapropoxy—;
- (5) an interlayer; and
- (6) a yellow layer containing "Coupler 4": 1-Imidazolidineacetamide, N-(5-((2-(2,4-bis (1,1-dimethylpropyl)phenoxy)-1-oxobutyl)amino)-2-chlorophenyl)—.alpha.—(2,2-dimethyl-1-oxo-propyl)-4-ethoxy-2,5-dioxo-3-(phenylmethyl)—.

In a reversal medium, the magenta coupler of the invention could be used to replace all or part of the magenta coupler in a photographic element such as one comprising a support and bearing the following layers from top to bottom:

- (1) one or more overcoat layers;
- (2) a nonsensitized silver halide containing layer;
- (3) a triple-coat yellow layer pack with a fast yellow layer containing "Coupler 1": Benzoic acid, 4-(1-((2-chloro-5-((dodecylsulfonyl)amino)phenyl)amino)carbonyl)-3,3-dimethyl-2-oxobutoxy)-, 1-methylethyl ester; a mid yellow layer containing Coupler 1 and "Coupler 2": Benzoic acid, 4-chloro-3-[[2-[4-ethoxy-2,5-dioxo-3-(phenylmethyl)-1-imidazolidinyl]-4,4-dimethyl-1,3-dioxopen-tyl]amino]-, dodecylester; and a slow yellow layer also containing Coupler 2;
- (4) an interlayer;
- (5) a layer of fine-grained silver;
- (6) an interlayer;
- (7) a triple-coated magenta pack with a fast magenta layer containing "Coupler 3": 2-Propenoic acid, butyl ester, polymer with N-[1-(2,5-dichlorophenyl)-4,5-dihydro-5-oxo-1H-pyrazol-3-yl]-2-methyl-2-propenamide; "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)-; and "Coupler 5": Benzamide, 3-(((2,4-bis(1,1-dimethylpropyl)phenoxy)acetyl)amino)-N-(4,5-dihydro-5-oxo-1-(2,4,6-trichlorophenyl)-1H-pyrazol-3-yl)-; and containing the stabilizer 1,1'-Spirobi(1H-indene), 2,2',3,3'-tetrahydro-3,3',3'-tetramethyl-5,5', 6,6'-tetrapropoxy-; and in the slow magenta layer Couplers 4 and 5 with the same stabilizer;
- (8) one or more interlayers possibly including fine-grained nonsensitized silver halide;
- (9) a triple-coated cyan pack with a fast cyan layer containing "Coupler 6": Tetradecanamide, 2-(2-cyanophenoxy)-N-(4-((2,2,3,3,4,4,4-heptafluoro-1-oxobutyl)amino)-3-hydroxyphenyl)-; a mid cyan containing "Coupler 7": Butanamide, N-(4-((2-(2,4-bis(1,1-dimethylpropyl)phenoxy)-1-oxobutyl)amino)-2-hydroxyphenyl)- 2,2,3,3,4,4,4-heptafluoro- and "Coupler 8": Hexanamide, 2-(2,4-bis(1,1-dimethylpropyl)phenoxy)-N-(4-((2,2,3,3,4,4,4-heptafluoro-1-oxobutyl)amino)-3-hydroxyphenyl)-;
- (10) one or more interlayers possibly including fine-grained nonsensitized silver halide; and
- (11) an antihalation layer.

If desired, the photographic element can be used in conjunction with an applied magnetic layer as described in *Research Disclosure*, November 1992, Item 34390 published by Kenneth Mason Publications, Ltd., Dudley Annex, 12a North Street, Emsworth, Hampshire PO10 7DQ, ENGLAND.

In the following discussion of suitable materials for use in the emulsions and elements of this invention, reference will be made to *Research Disclosure*, December 1989, Item No. 308119, available as described above which will be identified hereafter by the term "Research Disclosure." The contents of the *Research Disclosure*, including the patents and publications referenced therein, are incorporated herein by reference, and the Sections hereafter referred to are Sections of the *Research Disclosure*.

The silver halide emulsions employed in the elements of this invention can be either negative-working or positive-working. Suitable emulsions and their preparation as well as methods of chemical and spectral sensitization are described in Sections I through IV. Color materials and development modifiers are described in Sections V and XXI. Vehicles are described in Section IX, and various additives such as brighteners, antifog-gants, stabilizers, light absorbing and scattering materials, hardeners, coating aids, plasticizers, lubricants and matting agents are described, for example, in Sections V, VI, VIII, X, XI, XII, and XVI. Manufacturing methods are described in Sections XIV and XV, other layers and supports in Sections XIII and XVII, processing methods and agents in Sections XIX and XX, and exposure alternatives in Section XVIII.

Preferred color developing agents are p-phenylenediamines. Especially preferred are:

- 4-amino N,N-diethylaniline hydrochloride,
- 4-amino-3-methyl-N,N-diethylaniline hydrochloride,
- 4-amino-3-methyl-N-ethyl-N-(b-(methanesulfonamido) ethyl)aniline sesquisulfate hydrate,
- 4-amino-3-methyl-N-ethyl-N-(b-hydroxyethyl)aniline sulfate,
- 4-amino-3-b-(methanesulfonamido)ethyl-N,N-diethylaniline hydrochloride and
- 4-amino-N-ethyl-N-(2-methoxyethyl)-m-toluidine di-p-toluene sulfonic acid.

With negative working silver halide a negative image can be formed. Optionally positive (or reversal) image can be formed.

The coupler described herein may be used in combination with other classes of image couplers such as 3-acylamino- and 3-anilino-5-pyrazolones and heterocyclic couplers (e.g. pyrazoloazoles) such as those described in EP 285,274; U.S. Pat. No. 4,540,654; EP 119,860, or with other 5-pyrazolone couplers containing different ballasts or coupling-off groups such as those described in U.S. Pat. No. 4,301,235; U.S. Pat. No. 4,853,319 and U.S. Pat. No. 4,351,897. The coupler may also be used in association with yellow or cyan colored couplers (e.g. to adjust levels of interlayer correction) and with masking couplers such as those described in EP 213,490; Japanese Published Application 58-172,647; U.S. Pat. No. 2,983,608; German Application DE 2,706,117C; U.K. Patent 1,530,272; Japanese Application A-113935; U.S. Pat. No. 4,070,191 and German Application DE 2,643,965. The masking couplers may be shifted or blocked.

Coupling-off groups are well known in the art. Such groups can determine the equivalency of the coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, development acceleration or inhibition, bleach acceleration or inhibition, electron transfer facilitation, color correction and the like.

Representative classes of coupling-off groups include chloro, alkoxy, aryloxy, heteroaryloxy, sulfonyloxy, acyloxy, acyl, heterocyclyl, sulfonamido, mercaptotetrazole, mercaptopropionic acid, phosphonyloxy anylthio, and arylazo. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in U.K. Patents

and published application Nos. 1,466,728, 1,531,927, 1,533,039, 2,006,755A and 2,017,704A, the disclosures of which are incorporated herein by reference.

The magenta coupler described herein may be used in combination with other classes of magenta image couplers such as 3-acylamino-5-pyrazolones and heterocyclic couplers (e.g. pyrazoloazoles) such as those described in EP 285,274; U.S. Pat. No. 4,540,654; EP 119,860, or with other 5-pyrazolone couplers containing different ballasts or coupling-off groups such as those described in U.S. Pat. No. 4,301,235; U.S. Pat. No. 4,853,319 and U.S. Pat. No. 4,351,897. The coupler may also be used in association with yellow or cyan colored couplers (e.g. to adjust levels of interlayer correction) and with masking couplers such as those described in EP 213,490; Japanese Published Application 58-172,647; U.S. Pat. No. 2,983,608; German Application DE 2,706,117C; U.K. Patent 1,530,272; Japanese Application A-113935; U.S. Pat. No. 4,070,191 and German Application DE 2,643,965. The masking couplers may be shifted or blocked.

The couplers may also be used in association with materials that accelerate or otherwise modify the processing steps e.g. of bleaching or fixing to improve the quality of the image. Bleach accelerators described in EP 193,389; EP 301,477; U.S. Pat. No. 4,163,669; U.S. Pat. No. 4,865,956; and U.S. Pat. No. 4,923,784 are particularly useful. Also contemplated is use of the coupler in association with nucleating agents, development accelerators or their precursors (UK Patent 2,097,140; U.K. Patent 2,131,188); electron transfer agents (U.S. Pat. No. 4,859,578; U.S. Pat. No. 4,912,025); antifogging and anti color-mixing agents such as derivatives of hydroquinones, aminophenols, amines, gallic acid; catechol; ascorbic acid; hydrazides; sulfonamidophenols; and non color-forming couplers.

The couplers may also be used in combination with filter dye layers comprising colloidal silver sol or yellow and/or magenta filter dyes, either as oil-in-water dispersions, latex dispersions or as solid particle dispersions. Additionally, they may be used with "smearing" couplers (e.g. as described in U.S. Pat. No. 4,366,237; EP 96,570; U.S. Pat. No. 4,420,556; and U.S. Pat. No. 4,543,323.) Also, the couplers may be blocked or coated in protected form as described, for example, in Japanese Application 61/258,249 or U.S. Pat. No. 5,019,492.

The coupler may further be used in combination with image-modifying compounds such as "Developer Inhibitor-Releasing" compounds (DIR's). DIR's useful in conjunction with the couplers of the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063; DE 2,937,127; DE 3,636,824; DE 3,644,416 as well as the following European Patent Publications: 272,573; 335,319; 336,411; 346, 899; 362, 870; 365,252; 365,346; 37,3382; 376,212; 377,463; 378,236; 384,670; 396,486; 401,612; 401,613.

Such compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174

5 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include 10 a timing moiety or chemical switch which produces a delayed release of inhibitor. Examples of typical inhibitor moieties are: oxazoles, thiazoles, diazo, triazoles, 15 oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptothiazoles, mercaptotriazoles, mercaptooxadiazoles, mercaptodiazoles, mercaptooxathiazoles, telleurotetrazoles or benzisodiazoles. In a preferred embodiment, the inhibitor moiety or group is selected from the following formulas:



wherein R<sub>I</sub> is selected from the group consisting of straight and branched alkyls of from 1 to about 8 carbon atoms, benzyl and phenyl groups and said groups containing at least one alkoxy substituent; R<sub>II</sub> is selected from R<sub>I</sub> and —SR<sub>I</sub>; R<sub>III</sub> is a straight or branched alkyl group of from 1 to about 5 carbon atoms and m is from 1 to 3; and R<sub>IV</sub> is selected from the group consisting of hydrogen, halogens and alkoxy, phenyl and carbonamido groups, —COOR<sub>V</sub> and —NHCOOR<sub>V</sub> wherein R<sub>V</sub> is selected from substituted and unsubstituted alkyl and aryl groups.

Although it is typical that the coupler moiety included in the developer inhibitor-releasing coupler forms an image dye corresponding to the layer in which

it is located, it may also form a different color as one associated with a different film layer. It may also be useful that the coupler moiety included in the developer inhibitor-releasing coupler forms colorless products and/or products that wash out of the photographic material during processing (so-called "universal" couplers). 5

As mentioned, the developer inhibitor-releasing coupler may include a timing group which produces the time-delayed release of the inhibitor group such as 10 groups utilizing the cleavage reaction of a hemiacetal (U.S. Pat. No. 4,146,396; Japanese Applications 60-249148; 60-249149); groups using an intramolecular nucleophilic substitution reaction (U.S. Pat. No. 4,248,962); groups utilizing an electron transfer reaction 15 along a conjugated system (U.S. Pat. No. 4,409,323; 4,421,845; Japanese Applications 57-188035; 58-98728; 58-209736; 58-209738) groups utilizing ester hydrolysis (German Patent Application (OLS) No. 2,626,315; groups utilizing the cleavage of imino ketals (U.S. Pat. 20 No. 4,546,073); groups that function as a coupler or reducing agent after the coupler reaction (U.S. Pat. No. 4,438,193; U.S. Pat. No. 4,618,571) and groups that combine the features described above. It is typical that the timing group or moiety is of one of the formulas: 25



wherein IN is the inhibitor moiety, Z is selected from the group consisting of nitro, cyano, alkylsulfonyl; sulfamoyl ( $-\text{SO}_2\text{NR}_2$ ); and sulfonamido ( $-\text{NRSO}_2\text{R}$ ) groups; n is 0 or 1; and  $\text{R}_{VI}$  is selected from the group consisting of substituted and unsubstituted alkyl and phenyl groups. The oxygen atom of each timing group is bonded to the coupling-off position of the respective coupler moiety of the DIAR.

Suitable developer inhibitor-releasing couplers for use in the present invention include, but are not limited to, the following: 30



-continued





-continued

D7



D8

It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire PO101 7DQ, England, incorporated herein by reference. Materials of the invention may be coated on pH adjusted support as described in U.S. Pat. No. 4,917,994; with epoxy solvents (EP 0 164 961); with nickel complex stabilizers (U.S. Pat. Nos. 4,346,165; U.S. Pat. No. 4,540,653 and U.S. Pat. No. 4,906,559 for example); with ballasted chelating agents such as those in U.S. Pat. No. 4,994,359 to reduce sensitivity to polyvalent cations such as calcium; and with stain reducing compounds such as described in U.S. Pat. No. 5,068,171 and U.S. Pat. No. 5,096,805. Other compounds useful in combination with the invention are disclosed in Japanese Published Applications 83-09,959; 83-62,586; 90-072,629; 90-072,630; 90-072,632; 40 90-072,633; 90-072,634; 90-077,822; 90-078,229; 90-078,230; 90-079,336; 90-079,338; 90-079,690; 90-079,691; 90-080,487; 90-080,489; 90-080,490; 90-080,491; 90-080,492; 90-080,494; 90-085,928; 45 90-086,669; 90-086,670; 90-087,361; 90-087,362; 90-087,363; 90-087,364; 90-088,096; 90-088,097; 90-093,662; 90-093,663; 90-093,664; 90-093,665; 50 90-093,666; 90-093,668; 90-094,055; 90-094,056; 90-101,937; 90-103,409; 90-151,577.

Especially useful in this invention are tabular grain silver halide emulsions. Specifically contemplated tabular grain emulsions are those in which greater than 50 percent of the total projected area of the emulsion grains are accounted for by tabular grains having a 60

thickness of less than 0.3 micron (0.5 micron for blue sensitive emulsion) and an average tabularity (T) of greater than 25 (preferably greater than 100), where the term "tabularity" is employed in its art recognized usage as

$$T = ECD/t^2$$

where

ECD is the average equivalent circular diameter of the tabular grains in microns and  
t is the average thickness in microns of the tabular grains.

The average useful ECD of photographic emulsions can range up to about 10 microns, although in practice emulsion ECD's seldom exceed about 4 microns. Since both photographic speed and granularity increase with increasing ECD's, it is generally preferred to employ the smallest tabular grain ECD's compatible with achieving aim speed requirements.

Emulsion tabularity increases markedly with reductions in tabular grain thickness. It is generally preferred that aim tabular grain projected areas be satisfied by thin ( $t < 0.2$  micron) tabular grains. To achieve the lowest levels of granularity it is preferred that aim tabular grain projected areas be satisfied with ultrathin ( $t < 0.06$  micron) tabular grains. Tabular grain thicknesses typically range down to about 0.02 micron. However, still lower tabular grain thicknesses are contemplated. For example, Daubendiek et al U.S. Pat. No. 4,672,027 reports a 3 mole percent iodide tabular grain silver bro-

moiodide emulsion having a grain thickness of 0.017 micron.

As noted above tabular grains of less than the specified thickness account for at least 50 percent of the total grain projected area of the emulsion. To maximize the advantages of high tabularity it is generally preferred that tabular grains satisfying the stated thickness criterion account for the highest conveniently attainable percentage of the total grain projected area of the emulsion. For example, in preferred emulsions tabular grains satisfying the stated thickness criteria above account for at least 70 percent of the total grain projected area. In the highest performance tabular grain emulsions tabular grains satisfying the thickness criteria above account for at least 90 percent of total grain projected area.

Suitable tabular grain emulsions can be selected from among a variety of conventional teachings, such as those of the following: *Research Disclosure*, Item 22534, January 1983, published by Kenneth Mason Publications, Ltd., Emsworth, Hampshire P010 7DD, England; U.S. Pat. Nos. 4,439,520; 4,414,310; 4,433,048; 4,643,966; 4,647,528; 4,665,012; 4,672,027; 4,678,745; 4,693,964; 4,713,320; 4,722,886; 4,755,456; 4,775,617; 4,797,354; 4,801,522; 4,806,461; 4,835,095; 4,853,322; 4,914,014; 4,962,015; 4,985,350; 5,061,069 and 5,061,616.

The emulsions can be surface-sensitive emulsions, i.e., emulsions that form latent images primarily on the surfaces of the silver halide grains, or internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent.

Photographic elements can be exposed to actinic radiation, typically in the visible region of the spectrum, to form a latent image and then processed to form a visible dye image. Processing to form a visible dye image includes the step of contacting the element with a color developing agent to reduce developable silver halide and oxidize the color developing agent. Oxidized color developing agent in turn reacts with the coupler to yield a dye.

With negative-working silver halide, the processing step described above provides a negative image. The described elements can be processed in the known C-41 color process as described in, for example, the British Journal of Photography Annual of 1982, pages 209-211 and 1988, pages 191-198 or in known processes for processing color photographic papers, such as the known RA-4 process of Eastman Kodak Company. The described elements are optionally processed in the known color processes for processing color print papers, such as the processes described in the British Journal of Photography Annual of 1988, pages 198-199. To provide a positive (or reversal) image, the color development step can be preceded by development with a non-chromogenic developing agent to develop exposed silver halide, but not form dye, and then uniformly fogging the element to render unexposed silver halide, but not form dye, and then uniformly fogging the element to render unexposed silver halide developable. Alternatively, a direct positive emulsion can be employed to obtain a positive image.

Development is followed by the conventional steps of bleaching, fixing, or bleach-fixing, to remove silver or silver halide, washing, and drying.

Suitable stabilizers for the photographic elements of this invention include the following:



25



26



S-10 5

S-11 10

S-12 15

S-13 20

S-14 25

S-15 30

S-16 35

S-17 40

S-18 45

S-19 50

S-20 55

S-21 60

S-22 65

**SYNTHESIS OF COUPLERS**

The intermediates and the final couplers exhibited satisfactory  $^1\text{H}$  NMR (300 MHz,  $\text{CDCl}_3$ ) and combustion analysis. Chromatographic purifications were accomplished by flash chromatography on silica gel. Couplers were homogeneous (TLC) in solvent systems of different polarity. Removal of solvents involved evaporation at ca. 20 mmHg on a rotary evaporator. When inert or dry atmosphere is required, the manipulations were carried out in either nitrogen or argon atmosphere. The solvents used for the reaction were reagent grade, further dried over molecular sieves.

6-tert-Butyl-amine with a-Methyl Branched Linking Group



-continued

6-tert-Butyl-amine with a-Methyl Branched Linking Group



## Synthesis of 2-Methyl-3-N-Pthalimidopropionitrile(B)

A 1-L flask, equipped with a magnetic stirring bar was charged with phthalimide (1.17 moles), dry N,N-dimethylformamide (DMF, 200 mL), and methacrylonitrile (157 g, 2.34 moles). To this well stirred mixture was added triton B (23.4 mL, 40% in methanol.) The resulting yellow mixture was carefully brought to a gentle reflux (~110° C.), which turned red with time. The mixture was stirred for 18 hr as monitored by TLC to completion (dichloromethane:methanol, 2:1). The resulting mixture was cooled and poured into 2.5-L of crushed ice-water mixture. The orange solid was filtered. The solid was recrystallized from hot isopropyl alcohol (1.4-L). The white solid was filtered, first washed with a 2:1 mixture of cold isopropanol+water,

and finally with ethanol and dried to afford 187 g (75% yield) of B.

## Synthesis of Imidate (C)

5 A 1-L flask equipped with a magnetic stirring bar was dried (heat-gun) and cooled under a stream of argon. The flask was charged with nitrile (B, 50 g, 234 mmoles), anhydrous methanol (15 g, 468 mmol) and dichloromethane/ether mixture (100 mL). The mixture 10 was cooled to -10° C. (ice-acetone bath) followed by moderately bubbled in anhydrous hydrogen chloride gas for a period of 1 hr. Tetrahydofuran (THF, 50 mL) was added. The resulting mixture was stoppered and kept at 0 to 5° C. overnight. Evaporation of most of the 15 solvent under argon resulted in a white precipitation. To this precipitate was added dry chloroform (150 mL) which was vigorously stirred under nitrogen. The precipitate was quickly filtered, washed with chloroform (100 mL) and dried at -10° to 0° C. under nitrogen to 20 furnish the desired imidate (C, 60 g, 90%).

## Reaction of 3-Amino-4-Chloro-5-tert-Butylpyrazole

A magnetically stirred 2-L flask was dried with a heat gun and cooled under a dry stream of argon. The flask was charged with the above synthesized imidate (C, 95 g 336 mmol) and acetonitrile (900 mL), dried over 4A molecular sieves; 3-amino-4-chloro-5-tert-butylpyrazole (58.34 g, 336 mmol) was added, and the resulting mixture was heated (60-70° C. under argon for a 25 period of 2 hr to completion. On cooling a voluminous white precipitate was formed. The reaction mixture was cooled at about 0° C. (ice) and the yellow solid filtered, 30 washed with acetonitrile and dried to afford the amidine. This was further purified by triturating in ether to 35 furnish the desired amidine (F, 92.1 g, 65%).

## Reaction of Amidine with Hydroxylamine.hydrochloride

To a magnetically stirred mixture of amidine (212 40 mmol) in a mixture of methanol (500 mL) and water (700 mL) was added; hydroxylamine hydrochloride and anhydrous sodium acetate (424 mmol). The resulting mixture was gently refluxed for 2.5 hr to essential completion (TLC, CH<sub>2</sub>Cl<sub>2</sub>:MeOH, 9:2). The mixture was 45 cooled to about 0° C. (ice), and the precipitate was filtered. It was washed several times with water and dried to give a light yellow solid (76 g, 86% yield).

## Reaction of Oxime with p-Fluorobenesulfonyl Chloride

To a magnetically stirred mixture of the above oxime (65 g, 165 mmol) in sufficient tetrahydrofuran (450 mL) 50 solvent was added triethylamine (32.8 g, 324 mmol). The resulting mixture was cooled to 0° C. (ice-bath) and 4-fluorobenesulfonyl chloride (932.8 g, 169 mmol) was added in installments over a period of 10 min. Examination of the reaction by TLC (CH<sub>2</sub>Cl<sub>2</sub>:MeOH, 15:1) revealed the completion of the reaction. The mixture was poured into crushed ice. Precipitated p-fluorobenesulfonic acid was filtered and the aqueous layer extracted with 3×200 mL of ether. The combined extracts were dried (MgSO<sub>4</sub>). Removal of the volatiles furnished the p-fluorobenesulfonate of the oxime(G) as red viscous liquid (89 g, 98% crude yield).

## Cyclization of the Oxime-Sulfonate

The crude oxime-sulfonate was dissolved in anhydrous methanol (250 mL) and dry pyridine (12.5 g, 158

mmol) was added. The mixture was gently refluxed for 1 hr. The mixture was poured into crushed ice. The solid was filtered and further purified by trituration with methanol to provide the desired N-phthaloyl blocked bicyclic-pyrazolo-amine intermediate as a creamy white solid (H, 23.8 g, 40% yield).  $^1\text{H}$  NMR ( $\text{CDCl}_3$ ) was consistent with the structure.

Deblocking N-Phthaloyl Blocked bicyclic pyrazolo-Amine

To N-phthaloyl blocked bicyclicpyrazolo-amine derivative (22 g, 57 mmol) in absolute ethanol (500 mL) was added anhydrous hydrazine (3.66 g, 114 mmol). The mixture was stirred at room temperature (2.5 hr). Then the mixture was refluxed for 1 hr to completion (TLC,  $\text{CH}_2\text{Cl}_2:\text{MeOH}$ , 9:2 and  $\text{CH}_2\text{Cl}_2:\text{EtOAc}$ , 9:4). The mixture was filtered warm to remove the excess phthaloyl hydrazide and the resulting filtrate on cooling furnished the bicyclic-pyrazolo-amine (I). The amine was further purified by washing the precipitate with ice-cold water.



A 250-mL flask equipped with a magnetic stirring bar and addition funnel was charged with the bicyclic-pyrazolo-amine (2.55 g, 10 mmol), THF (50 mL), and N,N-dimethylaniline (1.8 g, 14 mmol). To this well stirred slurry was added 2-(m-pentadecylphenoxy)butyryl chloride (5 g, 12 mmol) dissolved in THF(25 mL). The reaction was monitored to completion (TLC,  $\text{CH}_2\text{Cl}_2:\text{EtOAc}$ , 9:2). The mixture was poured into crushed-ice and hydrochloric acid (pH 3-4). The gummy white solid was extracted with ethyl acetate and the combined extracts were dried ( $\text{MgSO}_4$ ). Removal of the solvents furnished 7.5 g of the crude coupler as viscous oil. The crude coupler was purified by flash chromatography to give the desired coupler as a glassy solid (4.4 g, 70% yield).

25 To a solution of the ballast acid chloride (7.67 g, 14 mmol) in dry dichloromethane (25 mL), maintained at 25° C. was added 2.14 g, 17 mmol of oxalyl chloride through the addition funnel. This was followed by the addition of N,N-dimethylformamide (DMF, 0.2 mL) to serve as the catalyst. The mixture was stirred at 40° C. to completion (30 min, TLC analysis of the methyl ester by quenching in dry methanol, ligroin 950:EtOAc., 9:1). 30 The volatiles were removed to furnish the acid chloride as a yellow liquid.

35 To a well stirred mixture of pyrazolotriazole-amine (3 g, 11.7 mmol) in THF (75 mL) and N,N-dimethylaniline (1.85 g, 15 mmol) at 0° C. (ice-bath) was added the acid chloride dissolved in THF (25 mL). The reaction was monitored to completion (TLC,  $\text{CH}_2\text{Cl}_2:\text{EtOAc}$ , 9:4). The mixture was poured into a mixture of crushed-ice and hydrochloric acid (pH 4). The solid was filtered and further purified by dissolving in hot acetonitrile-butyronitrile mixture to afford the coupler (6.5 g); mp 162-164° C. Anal Calcd. for  $\text{C}_{43}\text{H}_{64}\text{C}_1\text{N}_5\text{O}_4\text{S}$ : C, 66.00; H, 8.24; N, 8.95. Found: C, 65.91; H, 8.77; N, 8.16;

Preparation of Photographic Elements

45 Dispersions of the couplers were prepared in the following manner. The quantities of each component are found in Table I. In one vessel, the coupler, stabilizer (2,2',3,3'-tetrahydro-3,3,3',3'-tetramethyl-5,5',6,6'-tetrapropoxy-1,1'-spirobi[1H-indene]), coupler solvent 50 (diethyl dodecanoate), and ethyl acetate were combined and warmed to dissolve. In a second vessel, the gelatin, Alkanol XC™ (E. I. DuPont Co.) and water were combined and warmed to about 40° C. The two mixtures were mixed together and passed three times through a 55 Gaulin colloid mill. The ethyl acetate was removed by evaporation and water was added to restore the original weight after milling.

TABLE I

| Dispersion No. | Coupler No. | Grams Coupler | Grams Stabilizer | Grams Coupler Solvent | Grams Ethyl Acetate | Grams 12.5% Gelatin | Grams Alkanol XC (10%) | Grams Water |
|----------------|-------------|---------------|------------------|-----------------------|---------------------|---------------------|------------------------|-------------|
| 1              | M-1         | 0.804         | 0.402            | 1.206                 | 2.413               | 19.20               | 2.40                   | 13.57       |
| 2              | M-2         | 1.002         | 0.501            | 1.502                 | 3.005               | 19.20               | 2.40                   | 12.39       |
| 3              | C-1         | 0.750         | 0.375            | 1.126                 | 2.251               | 19.20               | 2.40                   | 13.90       |
| 4              | C-2         | 0.732         | 0.366            | 1.099                 | 2.197               | 19.20               | 2.40                   | 14.01       |
| 5              | C-3         | 0.786         | 0.393            | 1.179                 | 2.359               | 19.20               | 2.40                   | 13.68       |
| 6              | C-4         | 1.005         | 0.503            | 1.508                 | 3.016               | 16.20               | 2.40                   | 12.37       |

Dispersion 7 was composed of comparison coupler C-5 (8.73% by weight), 3,4-dihydro-2,2-dimethyl-4-(1-methylethyl)-7-octyl-2H-1-benzopyran-6-ol (3.714%), 2,5-di-sec-dodecylhydroquinone (0.873%), dibutyl phthalate (4.454%) and gelatin (8.69%).

Comparison Coupler C-1



Comparison Coupler C-2



Comparison Coupler C-3



Comparison Coupler C-4



Comparison Coupler C-5



The photographic elements of Examples 1, 2, 3, 5, 6, 7, 9, 10, 12, 13, 14, 16, 17, 18, 20, 21, 23, and 24 were prepared by coating the following layers in the order listed on a resin-coated paper support:

|                                                             | Developer                                                                                              |          |
|-------------------------------------------------------------|--------------------------------------------------------------------------------------------------------|----------|
| 1st Layer                                                   | Triethanolamine                                                                                        | 12.41 g  |
| Gelatin                                                     | Blankophor REU™ (Mobay Corp.)                                                                          | 2.30 g   |
| <u>2nd Layer</u>                                            | Lithium polystyrene sulfonate (30%)                                                                    | 0.30 g   |
| Gelatin                                                     | N,N-Diethylhydroxylamine (85%)                                                                         | 5.40 g   |
| Coupler Dispersion                                          | Lithium sulfate                                                                                        | 2.70 g   |
| Green-sensitized AgCl emulsion                              | N-{2-[(4-amino-3-methylphenyl)ethylamino]ethyl}-methanesulfonamide, sesquisulfate                      | 5.00 g   |
| <u>3rd Layer</u>                                            | 1-Hydroxyethyl-1,1-diphosphonic acid (60%)                                                             | 0.81 g   |
| Gelatin                                                     | Potassium carbonate, anhydrous                                                                         | 21.16 g  |
| 2-(2H-benzotriazol-2-yl)-4,6-bis-(1,1-dimethylpropyl)phenol | Potassium chloride                                                                                     | 1.60 g   |
| Tinuvin 326™ (Ciba-Geigy)                                   | Potassium bromide                                                                                      | 7.00 mg  |
| <u>4th Layer</u>                                            | Water to make                                                                                          | 1.00 L   |
| Gelatin                                                     | pH @ 26.7° C. adjusted to 10.4 ± 0.05                                                                  |          |
| Bis(vinylsulfonylmethyl) ether                              | <u>Bleach-Fix</u>                                                                                      |          |
|                                                             | Solution of anunonium thiosulfate (56.4%) + Ammonium sulfite (4%)                                      | 127.40 g |
|                                                             | Sodium metabisulfite                                                                                   | 10.00 g  |
|                                                             | Acetic acid (glacial)                                                                                  | 10.20 g  |
|                                                             | Solution of ammonium ferric ethylenediaminetetraacetate (44%) + ethylenediaminetetraacetic acid (3.5%) | 110.40 g |
|                                                             | Water to make                                                                                          | 1.00 L   |
|                                                             | pH @ 26.7° C. adjusted to 6.7                                                                          |          |

The photographic elements for Examples 4, 8, 11, 15, 19, 22, and 25 were prepared in the same manner except that the amount of coupler dispersion in the 2nd layer

was  $5.6 \times 10^{-4}$  mole coupler/m<sup>2</sup> and the amount of AgCl emulsion in the 2nd layer was 0.29 g Ag/m<sup>2</sup>

The photographic elements were given stepwise exposures to green light and processed as follows at 35° C.:

Developer: 45 seconds

Bleach-Fix: 45 seconds

Wash (running water): 1 minute, 30 seconds

The developer and bleach-fix were of the following compositions:



4. A photographic element as in claim 1, wherein L contains at least one alkylene group in the connecting chain.

5. A photographic element as in claim 1, wherein R is selected from the group consisting of t-butyl, 1,1,3,3-methylbutyl, t-pentyl, and adamantyl.

6. A photographic element as in claim 1, wherein Ar is a phenyl group.

7. A photographic element as in claim 6, wherein Y is —O—.

5 8. A process of forming a dye image in an exposed photographic element as defined in claim 1, said process comprising developing the photographic element in the presence of a color developing agent.

\* \* \* \* \*

10

15

20

25

30

35

40

45

50

55

60

65